

# United States Patent Office

3,320,315  
Patented May 16, 1967

1

3,320,315

## BIS-( $\beta$ -OXYPROPIONAMIDO)-ALKYNES

Jack L. Towle, East Cleveland, and Dale G. Block, Cleveland, Ohio, assignors, by mesne assignments, to Kewanee Oil Company, Bryn Mawr, Pa., a corporation of Delaware  
No Drawing. Filed Aug. 31, 1964, Ser. No. 393,403  
6 Claims. (Cl. 260—561)

### ABSTRACT OF THE DISCLOSURE

The invention comprises new compounds having an acetylenic bond therein and suitable as additives in electroplating baths comprising the reaction product of an unsaturated carboxamide and an acetylene diol. The simplest of these compounds is prepared by the reaction of butynediol with acrylamide. More complex compounds are prepared by forming the ethylene oxide derivatives of the diol prior to the reaction with the unsaturated carboxamide.

This invention relates generally to triple bond-containing diamides useful as additives in electroplating baths. More particularly the invention relates to the reaction product of an unsaturated carboxamide and a triple bond-containing diol.

The reaction products comprising the present invention may be described as alkyneoxyalkanoic diamides and alkadiyneoxyalkanoic diamides. These compounds may be represented by the following general formula.

I.



wherein  $n$  is an integer ranging from 0 to 20 inclusive, A represents a member selected from the group consisting of ethylene ( $-\text{C}\equiv\text{C}-$ ) and diethynylene



and when  $n$  is 0 R represents hydrogen and R1 represents hydrogen and an alkyl radical having from 1 to 2 carbon atoms. When  $n$  is 1 to 20, R and R1 may represent hydrogen and an alkyl radical having from 1 to 2 carbon atoms, and Z represents a member selected from the group consisting of hydrogen, methyl and hydroxymethyl.

The compounds defined by Formula I above are prepared in good yields by the direct reaction of an acetylenic diol and an  $\alpha,\beta$ -ethylenically unsaturated amide. Advantageously, two moles of amide are reacted with one mole of the diol in the presence of a basic catalyst. Representative of the reaction is that between acrylamide and 1,4-butynediol which is illustrated by the following equation.



Compounds of the class defined by Formula I have been found to produce leveling when employed with an aqueous acid solution of nickel salts capable of supplying nickel ions such as, for instance, the familiar all chloride, all sulfate, sulfate-chloride or Watts type, nickel fluoroborate, nickel sulfamate types and combinations thereof. Moreover the diamides of the present invention

2

characteristically do not cause misplate or skipped areas on the article to be plated.

In general, the compounds of the present invention are advantageously employed as leviers in concentrations in the range of from about .005 g./l. to about 1.0 g./l. Within this broad concentration range there are three more limited ranges wherein the limits are determined by the type of cooperating additives employed with the leveler and by the type of nickel coating desired. When the compound is employed as a leveler alone in a nickel plating bath without the use of cooperating compounds, the compound preferably is present in the range of from about .005 g./l. to about 0.1 g./l. When the compound is employed as a leveler in a nickel plating bath containing cooperating compounds for purposes of obtaining a semi-bright nickel plate, the compound preferably is present in the range of from about .01 g./l. to about 0.3 g./l. When the compound is employed in a nickel plating bath containing cooperating compounds for purposes of obtaining a bright nickel plate, the compound preferably is present in the range of from about .05 g./l. to about 1.0 g./l.

Increased leveling and more uniform lustre are obtained with the instant compounds when they are employed in combination with a second cooperating compound. The cooperating compound is defined as a trihalo aldehyde or acetal or hemiacetal precursor thereof.

Specific examples of the cooperating compounds include 1,1 - diethoxy-2,2,2-trichloroethane, 1-hydroxy-1-ethoxy-2,2,2-trichloroethane, 1,1-dimethoxy-2,2,2-trichloroethane, 1-hydroxy-1-methoxy - 2,2,2 - trichloroethane, 1,1 - dimethoxy-2,2,2-triboromethane, trichloroethanal, and tribromoethanal.

In general, these cooperating compounds when present in the semi-bright plating solutions are employed advantageously in concentrations in the range of from about 0.01 gram per liter to about 2.0 grams per liter. Trichloroethanal, an especially useful cooperating compound, may be used to advantage in the semi-bright platings solution in concentrations in the range of from about 0.01 gram per liter to about 0.5 gram per liter, and preferably in the range of from about 0.03 gram per liter to about 0.1 gram per liter.

In general, the compounds of this invention are prepared by dissolving the acetylenic diol and the amide in a suitable solvent and adding the required amount of alkaline catalyst such as an aqueous solution of trimethyl benzyl ammonium hydroxide, aqueous potassium hydroxide or sodium tertiary butoxide. The quantity of catalyst required is in the range of from about 1 percent to about 20 percent by weight of the combined weights of the reactants. In addition to the catalysts mentioned, any agent capable of promoting a Michael reaction would serve in these reactions. Other suitable catalysts for use in carrying out the Michael reaction include alkali-metal alkoxides, -aryls and -amides.

The preferred solvent is tertiary butanol but other compounds free of hydrogen atoms capable of undergoing conjugate addition reactions may be used, such as dioxane, tetrahydrofuran, 1,2-dimethoxyethane and the like. The compound should be liquid at room temperature (25° C.) and substantially inert to the reactants and the catalysts.

The reaction takes place readily at temperatures in the range of from about 25° C. to about 100° C., although temperatures in the range of from about 40° C. to about 70° C. are preferred. The reaction period is not critical; periods ranging from 3 to 16 hours may be used, although most reactions are completed within periods ranging from 4 to 8 hours.

When the reaction is completed, the product may be isolated and purified by recrystallization from solvents such as methyl or ethyl alcohol.

## 3

Specific acetylenic diols suitable as reactants for preparing the compounds of the present invention include 3-hexyne-1,6-diol, 2-pentyne-1,5-diol, 2-butyne-1,4-diol and 2,4-hexadiyne-1,6-diol. These acetylenic diols are also advantageously reacted with up to 20 moles and preferably not more than 5 moles of ethylene oxide per hydroxyl group. These reaction products being diols themselves may be reacted with the  $\alpha,\beta$ -ethylenically unsaturated amide. The original diol may contain secondary hydroxyl groups which can be reacted with ethylene oxide. The hydroxyl groups preferably should be on the second or third carbon atom from the end of the alkyne chain. Moreover the original diol may be a tertiary diol if it is first reacted with ethylene oxide in the manner disclosed by K. D. Petrov and E. S. Laguchevu, Zhur. Obschhei Khim., 21, 1247 (1951), C.A. 46, 1959.

The amides employed have the general formula:



wherein Z is hydrogen, methyl or hydroxymethyl group.

Specific amides which have been found suitable for purposes of this invention are acrylamide, N-methylacrylamide and N-hydroxymethylacrylamide.

These following examples are given for purposes of illustration and not by way of limitation. All parts and percentages are by weight unless otherwise specified.

## EXAMPLE I

1,4-bis( $\beta$ -oxypropionamide)butyne-2

In a one liter 3-necked flask equipped with stirrer, thermometer and reflux condenser is placed 325 g. of tertiary butanol. The alcohol is heated to 40° C. and 43 g. (0.5 mole) 2-butyne-1,4-diol, 71.5 g. (1.01 moles) acrylamide and 7.2 g. of 40% aqueous potassium hydroxide is added in that order. The cloudy orange solution is filtered through Filter-cel and the clear orange filtrate heated with stirring at 45° C.-50° C. for eight hours. After one hour, the product begins to separate from solution and soon the reaction mixture is a thick cream-colored mass.

At the end of eight hours, the mixture is cooled to 30° C., filtered and the pale brown solid dried to constant weight in an oven at 80° C. The crude yield is 104 g. (91.2%) melting at 112° C.-118° C.

The crude product is dissolved in 325 g. of hot absolute methanol containing 1 g. of activated carbon, heated for 15 minutes and filtered. The orange filtrate is cooled to 20° C. and the crystals which separated are filtered and dried. The product weighs 74 g. (overall yield of 65%) and melts at 132° C. to 133° C. The elemental analysis, molecular weight determinations and infrared absorbencies of the product are as follows: Calculated for  $\text{C}_{10}\text{H}_{16}\text{N}_2\text{O}_4$ : C, 52.62; H, 7.07; N, 12.27; mol. wt. 228. Found: C, 53.00; H, 6.91; N, 12.29; mol. wt. ebullioscopic in ethanol, 228; in butanone, 232.

$\lambda_{\text{max}}^{\text{KBr}} (\mu)$  3.43, 3.47 ( $\text{CH}_2$ ); 2.98, 3.15 (amide NH); 6.02, 6.07, 6.20 (amide  $\text{C}=\text{O}$ ); 8.97, 9.22, 9.37 ( $\text{C}-\text{O}-\text{C}$ ).

## EXAMPLE II

1,4-bis( $\beta$ -oxypropionamide)butyne-2

A mixture of 28.4 g. (0.4 mole) of acrylamide, 17.2 g. (0.2 mole) of 1,4-butyne diol and 200 g. of tertiary butyl alcohol is stirred at 50° C. until a clear solution is obtained. To this is added a slurry of sodium tertiary-butoxide prepared from 2 g. of sodium and 24 g. of tertiary butyl alcohol and the mixture stirred at 45° C.-50° C. for eight hours and then allowed to stand at room temperature for an additional 10 hours. The resulting thick slurry is then added to 800 g. of ethyl ether, mixed thoroughly, and filtered. The crude product is recrystallized from anhydrous methanol to give 24.5 g. (63.3%) of 1,4-bis( $\beta$ -oxypropionamide)butyne-2, melting at 133° C.-134° C.

## 4

The infrared absorbancies are as follows:

$\lambda_{\text{max}}^{\text{KBr}} (\mu)$  3.43, 3.47 ( $\text{CH}_2$ ); 2.98, 3.15 (amide NH); 6.02, 6.07, 6.20 (amide  $\text{C}=\text{O}$ ); 8.97, 9.22, 9.37, ( $\text{C}-\text{O}-\text{C}$ )

## EXAMPLE III

1,4-bis( $N$ -methyl- $\beta$ -oxypropionamide)butyne-2

To 59.3 g. tertiary butanol is added 8.6 g. (0.1 mole) 1,4-butyne diol and then heated with agitation until solution is complete. At 35° C.-40° C. is added 17.0 (0.2 mole) N-methylacrylamide followed by 5.0 g. 50% aqueous benzyltrimethyl ammonium hydroxide (Triton B). A nitrogen atmosphere is provided and the temperature raised to 45° C.-50° C. and maintained at this temperature for a period of eight hours during which time the reaction mixture is continuously agitated. At the end of this time, the mixture is transferred to a separatory funnel and extracted with two 200 ml. portions of petroleum ether (B.P. 30° C.-60° C.) to remove the tertiary butanol. The brown oil that remains subsequent to the petroleum ether extraction partially crystallizes. The crystals that separate are washed free from the brown oil with successive 50 ml. portions of petroleum ether. The crystalline product collected is recrystallized from dioxane to give a product that melts at 104° C.-105° C. and weighs 7.0 g.

The infrared absorbancies are as follows:

$\lambda_{\text{max}}^{\text{KBr}} (\mu)$  3.35 ( $\text{CH}_2$ ); 3.35 (amide  $\text{N}-\text{CH}_3$ ); 3.00 (amide NH), 5.95, 6.07 (amide  $\text{C}=\text{O}$ ), 8.88, 9.24 ( $\text{C}-\text{O}-\text{C}$ ).

## EXAMPLE IV

1,6-bis( $\beta$ -oxypropionamide)hexadiyne-2,4

In a 500 ml. 3-necked flask equipped with a stirrer, thermometer and reflux condenser is placed a mixture of 11 g. (0.1 mole) 2,4-hexadiyne-1,6-diol, 14.3 g. (0.202 mole) acrylamide and 2.9 g. 40% aqueous benzyl trimethyl ammonium hydroxide (Triton B) in 148 g. tertiary butanol. The mixture is stirred at 45° C.-50° C. for eight hours and then allowed to stand at room temperature overnight. A small amount (1.5 g.) of black material is filtered off, and the clear deep red filtrate is slowly poured with stirring into one liter of ethyl ether. An orange brown gum separates but on further stirring solidifies to a solid brown mass. This solid is recrystallized twice from 95% ethanol to give gray plates (which turned purple on drying) melting at 129° C. to 134° C. A mixed melting point with 2,4-hexadiyne-1,6-diol (M.P. 110° C.-113° C.) is 80° C.-85° C. The compound is soluble in hot water, and the infrared spectrum showed characteristic frequencies for the ether and amide linkages.

The infrared absorbancies are as follows:

$\lambda_{\text{max}}^{\text{KBr}} (\mu)$  3.40, 3.50 ( $\text{CH}_2$ ), 2.90, 3.12 (amide NH), 5.88, 6.00 (amide  $\text{C}=\text{O}$ ), 9.08, 9.18 ( $\text{C}-\text{O}-\text{C}$ ).

## EXAMPLE V

1,4-bis( $N$ -hydroxymethyl- $\beta$ -oxypropionamide)butyne-2

A solution of 33.7 g. of 60% aqueous N-hydroxymethyl acrylamide, 8.6 g. 1,4-butyne diol and 5 g. of 40% aqueous benzyltrimethyl ammonium hydroxide (Triton B) in 34 g. tertiary butanol allowed to stand overnight at about 35°. The resulting thick paste is slurried twice with cold isopropyl alcohol and filtered. It is then recrystallized twice from 80% aqueous ethanol to give an almost white product melting at 160° C.-165° C.

The infrared absorbancies are as follows:

$\lambda_{\text{max}}^{\text{KBr}} (\mu)$  3.42, 3.47 ( $\text{CH}_2$ ); 2.88, 9.45, 14.30 (alkyl OH); 7.0 (amide NH); 6.02 (amide  $\text{C}=\text{O}$ ); 8.80, 9.10 ( $\text{C}-\text{O}-\text{C}$ ).

## EXAMPLES VI AND VII

As mentioned hereinbefore the unsaturated diols may be reacted with up to about 20 moles of ethylene oxide

per hydroxyl of the diol. The following examples give the preparation of such products.

*Ethylene oxide adduct of 2-butyne-1,4-diol*

Into a 1 liter 3-necked flask containing 354 grams of isopropanol is charged 14 grams of potassium hydroxide and 21.5 grams (0.25 mole) of 2-butyne-1,4-diol. 110.0 grams (2.5 mole) of ethylene oxide is then added to the flask, and the resulting solution turns a dark brown. After 5½ hours at reflux temperature the solution is cooled and filtered through a sintered glass filter, leaving practically no residue. With a second filtering through

10 pounds. The plating solution may also contain an antipitting agent, although the deposits may be suitable without the antipitting agent.

Sodium lauryl sulfate or other wetting agents such as the sodium sulfate derivative of 7-ethyl-2-methylundecanol-4 and the dihexyl ester of sodium sulfosuccinic acid and the like may be used as an antipitting agent.

Preferred concentration ranges for preferred compounds are given in the following table designated as Table I.

10 Specific examples of the electroplating solutions containing different cooperating additives are illustrated in the

TABLE I

|          |                                                                                                                                                     |                                                                   | Concentration Range  |                                                       |                                                 |
|----------|-----------------------------------------------------------------------------------------------------------------------------------------------------|-------------------------------------------------------------------|----------------------|-------------------------------------------------------|-------------------------------------------------|
|          |                                                                                                                                                     |                                                                   | Leveler alone, g./l. | Semi-Bright leveler plus cooperating compounds, g./l. | Bright leveler plus cooperating compound, g./l. |
| (1)----- | $\text{NH}_2\text{COCH}_2\text{CH}_2\text{OCH}_2\text{C}\equiv\text{C}-\text{CH}_2\text{OCH}_2\text{CH}_2\text{CONH}_2$ -----                       | 1,4-bis( $\beta$ -oxypropionamide)butyne-2.                       | .01-.04              | .03-.10                                               | .1-.5                                           |
| (2)----- | $\text{NH}_2\text{CO}(\text{CH}_2\text{CH}_2\text{O})_5\text{CH}_2\text{C}\equiv\text{CCH}_2\text{C}(\text{OCH}_2\text{CH}_2)_5\text{CONH}_2$ ----- | $\omega,\omega'$ -Dicarbamyl-1,4-bis [hexa(oxyethylene)]butyne-2. | .01-.04              | .03-.10                                               | .1-.5                                           |
| (3)----- | $\text{NH}_2\text{COCH}_2\text{CH}_2\text{OCH}_2\text{C}\equiv\text{C}-\text{C}\equiv\text{CCH}_2\text{OCH}_2\text{CH}_2\text{CONH}_2$ -----        | 1,6-bis( $\beta$ -oxypropionamide)hexadiyne-2,4.                  | .025-.1              | .05-.30                                               | .25-.7                                          |
| (4)----- | $\text{HOCH}_2\text{NHCOCH}_2\text{CH}_2\text{OCH}_2\text{C}\equiv\text{CCH}_2\text{OCH}_2\text{CH}_2\text{CONHCH}_2\text{OH}$ -----                | 1,4-bis(N-hydroxymethyl- $\beta$ -oxypropionamide)butyne-2.       | .01-.06              | .03-.20                                               | .1-1.0                                          |
| (5)----- | $\text{CH}_3\text{NHCOCH}_2\text{CH}_2\text{OCH}_2\text{C}\equiv\text{CCH}_2\text{OCH}_2\text{CH}_2\text{CONHCH}_3$ -----                           | 1,4-bis(N-methyl- $\beta$ -oxypropionamide)butyne-2.              | .01-.06              | .03-.20                                               | .1-1.0                                          |

activated carbon (Nuchar) the filtrate becomes light brown in color. The isopropanol is then stripped from the filtrated reaction mass leaving an oily light brown product. The resulting product is ethoxylated 2-butyne-1,4-diol having on the average about five moles of ethylene oxide per hydroxyl group.

Another ethylene oxide adduct of 2-butyne-1,4-diol is prepared following substantially the above procedure, but using 4 times as much ethylene oxide. The resulting product has substantially the same appearance as the product of Example VI but is more viscous.

EXAMPLES VIII AND IX

Basing the molecular weights of the products of Examples VI and VII on the amount of ethylene oxide used in the reaction, respective amounts of acrylamide are reacted with these products in accordance with the procedure outline in Example I. The resulting diamides may be represented by the general formula designated as I (supra) wherein  $n$  is 5 and 20 respectively for the two products.

The acetylenic diamides of the present invention advantageously may be used in a bath comprising—

(1) Water.

(2) A source of nickel ions comprising at least one nickel salt selected from the group consisting of: nickel sulfate, nickel chloride, nickel sulfamate and nickel fluoroborate.

(3) One of the hereinbefore-mentioned cooperating compounds.

(4) A wetting agent (optional).

An additional ingredient of the solution which is desirable is a buffering agent such as boric acid, formic acid, sodium formate and the like.

As mentioned hereinbefore the basic nickel-containing solutions advantageously contain one or more of the compounds of the present invention and preferably one or more of the hereinbefore mentioned cooperating com-

40 preceding table. It should be understood that the specific electroplating solutions may be employed with or without air agitation.

TABLE

|                                                 |         |     |
|-------------------------------------------------|---------|-----|
| $\text{NiSO}_4 \cdot 6\text{H}_2\text{O}$ ----- | oz./gal | 40  |
| $\text{NiCl}_2 \cdot 6\text{H}_2\text{O}$ ----- | oz./gal | 6   |
| $\text{H}_3\text{BO}_3$ -----                   | oz./gal | 5.5 |
| pH -----                                        |         | 4.0 |
| Temperature -----                               | ° F     | 140 |
| Current density -----                           | a.s.f.  | 45  |

(1) To the basic solution of Example 1 is added:



(2) To the basic nickel solution of Example 1 is added:



(3) A plating solution containing:

|                                                                        |         |      |
|------------------------------------------------------------------------|---------|------|
| Nickel fluoroborate -----                                              | oz./gal | 45   |
| Boric acid -----                                                       | oz./gal | 4    |
| pH -----                                                               |         | 3.0  |
| Temperature -----                                                      | ° F     | 100  |
| $\text{NH}_2\text{COCH}_2\text{CH}_2\text{OCH}_2\text{C}$ -----        | g./l.   | 0.07 |
| $\equiv\text{C}-\text{CH}_2\text{OCH}_2\text{CH}_2\text{CONH}_2$ ----- | g./l.   | 0.1  |
| Trichloroethanal -----                                                 | g./l.   | 0.1  |

(4) Plating solution containing:

|                                                                                       |         |     |
|---------------------------------------------------------------------------------------|---------|-----|
| Nickel sulfamate -----                                                                | oz./gal | 45  |
| Nickel chloride -----                                                                 | oz./gal | 1   |
| pH -----                                                                              |         | 4.0 |
| Temperature -----                                                                     | ° F     | 140 |
| $\text{NH}_2\text{COCH}_2\text{CH}_2\text{OCH}_2\text{C}$ -----                       | g./l.   | 0.2 |
| $\equiv\text{C}-\text{C}\equiv\text{CCH}_2\text{OCH}_2\text{CH}_2\text{CONH}_2$ ----- | g./l.   | 0.1 |
| Trichloroethanal -----                                                                | g./l.   | 0.1 |

While the foregoing electroplating baths are prepared in concentrations and employed at current densities for the electrodeposition thereof. When a bright nickel deposit is desired, the compound or leveling agent of the present invention should be employed in concentrations of from about .05 gram per liter to about 1.0 gram per liter. Moreover the compounds may advantageously be employed with the hereinbefore mentioned cooperating addition agents.

The compounds of the present invention have been found to be suitable for electrodepositing nickel upon any of the basis metals commonly employed in the electroplating art, such as, for example, iron, steel, copper, brass and zinc. It has been found, however, that the compounds (leveling addition agents) of this invention and particularly when the leveling addition agent of this invention is employed in conjunction with the cooperating addition agent enhanced nickel electrodeposits are obtained on zinc die castings. The zinc basis metal is, of course, preferably subjected to those pretreatment operations common to the art of electroplating prior to the deposition of nickel from the nickel plating bath of this invention. The coating of zinc basis metal with copper is commonly done prior to electrodeposition of nickel. In general, the degree of leveling obtained through the deposition of a semi-bright plate of this invention is from about 20 percent to about 50 percent for 1 mil deposits. The percentage of leveling is defined as—

$$100 \times \frac{\text{decrease in roughness due to plating}}{\text{initial roughness of basis metal}}$$

Where there is noticeable zinc contamination in the bath the compound prepared according to Example I particularly may be used; the tolerance of this compound for zinc is particularly high.

While specific examples of the invention have been set forth hereinabove, it is not intended that the invention be limited solely thereto but to include all of the variations and modifications falling within the scope of the appended claims.

What is claimed is:

1. A class of compounds represented by the following general formula:



wherein  $n$  is an integer ranging from 0 to 20 inclusive, A represents a member selected from the group consisting of ethynylene and diethynylene, and when  $n$  is 0, R represents hydrogen and  $R_1$  represents a member selected from the group consisting of hydrogen and alkyl having from 1 to 2 carbon atoms, and when  $n$  is 1 to 20, R and  $R_1$  represent a member selected from the group consisting of hydrogen and alkyl having from 1 to 2 carbon atoms, and Z represents a member selected from the group consisting of hydrogen, methyl and hydroxymethyl.

**2. The compound represented by the formula:**



3. The compound represented by the formula:



4. The compound represented by the formula:



5. The compound represented by the formula:



6. The compound represented by the formula:



No references cited.

ALEX MAZEL, *Primary Examiner.*

JOSEPH A. NARCAVAGE, *Assistant Examiner.*

40